



US005817809A

# United States Patent [19]

Begley et al.

[11] Patent Number: 5,817,809

[45] Date of Patent: Oct. 6, 1998

[54] **PHOTOGRAPHIC ELEMENT CONTAINING A COUPLER CAPABLE OF RELEASING A PHOTOGRAPHICALLY USEFUL GROUP THROUGH A TRIAZOLE GROUP**

[75] Inventors: **William James Begley**, Webster; **Frank D. Coms**; **Teh-Hsuan Chen**, both of Fairport, all of N.Y.

[73] Assignee: **Eastman Kodak Company**, Rochester, N.Y.

[21] Appl. No.: **923,842**

[22] Filed: **Sep. 4, 1997**

## Related U.S. Application Data

[62] Division of Ser. No. 733,373, Oct. 17, 1996, Pat. No. 5,709,987.

[51] **Int. Cl.<sup>6</sup>** ..... **C07D 413/12**; C07D 403/14; C07D 249/06

[52] **U.S. Cl.** ..... **544/132**; 548/144; 548/217; 548/251; 548/255

[58] **Field of Search** ..... 548/144, 217, 548/251, 255; 544/132

## [56] References Cited

### U.S. PATENT DOCUMENTS

4,861,701 8/1989 Burns et al. ..... 430/543  
5,035,988 7/1991 Nakamura et al. ..... 430/551

### FOREIGN PATENT DOCUMENTS

0 362 870 4/1990 European Pat. Off. .  
0 438 129 7/1991 European Pat. Off. .  
0 499 279 8/1992 European Pat. Off. .  
0 576 089 12/1993 European Pat. Off. .  
60-229 030 11/1985 Japan ..... 430/955

*Primary Examiner*—Fiona T. Powers  
*Attorney, Agent, or Firm*—Sarah Meeks Roberts

## [57] ABSTRACT

A photographic element comprising a support having situated thereon at least one silver halide emulsion layer, the element further comprising a photographic coupler represented by the formula



wherein

COUP is a coupler moiety having a coupling site to which  $\text{T}^1$  is attached;

$\text{T}^1$  is a timing or linking group which releases from COUP during processing and which functions by electron transfer down a conjugated or unconjugated chain, or by a nucleophilic displacement reaction, to release  $\text{T}^2$ ;  
 $\text{T}^2$  is a triazole timing or linking group which, after release from  $\text{T}^1$ , functions by a nucleophilic displacement reaction to release  $\text{T}^3$  or PUG and is represented by the formula:



wherein \*\* denotes the point of attachment to  $\text{T}^1$  and \*\*\* denotes the point of attachment to  $\text{T}^3$  or PUG;

$\text{R}^1$  is a hydrogen or halogen atom, or an aliphatic, carbocyclic, carbamoyl, sulfamoyl, carbonamido, sulfonamido, alkoxy carbonyl, alkyl or arylketo, alkyl or arylsulfo, sulfo, hydroxy, acyl, nitro, cyano, amino, alkoxy, alkoxyalkyl, aryloxy, aryloxyalkyl, thioalkoxy, thioalkoxyalkyl, thioaryloxy, thioaryloxyalkyl or heterocyclic group;

$\text{X}^2$  is a linking group which spatially relates a nitrogen atom of the triazole ring and  $\text{E}^2$  so that upon displacement of  $\text{T}^2$  from  $\text{T}^1$ ,  $\text{T}^2$  undergoes a nucleophilic displacement reaction with the formation of a three to eight membered ring and the cleavage of the bond between  $\text{E}^2$  and PUG or  $\text{T}^3$ ;

$\text{E}^2$  is an electrophilic group which is attached to  $\text{T}^3$  or PUG and which is displaced therefrom by said nucleophilic displacement reaction after  $\text{T}^2$  is displaced from  $\text{T}^1$ ;

$\text{T}^3$  is a timing or linking group attached to  $\text{E}^2$  which is released therefrom after  $\text{T}^2$  releases from  $\text{T}^1$ , and which functions by electron transfer down a conjugated or unconjugated chain, or by a nucleophilic displacement reaction, to release PUG;

b and c are independently selected from 0 or 1; and PUG is a photographically useful group.

**2 Claims, No Drawings**

## 1

**PHOTOGRAPHIC ELEMENT CONTAINING  
A COUPLER CAPABLE OF RELEASING A  
PHOTOGRAPHICALLY USEFUL GROUP  
THROUGH A TRIAZOLE GROUP**

This is a Divisional of application Ser. No. 08/733,373, filed Oct. 17, 1996, now U.S. Pat. No. 5,709,987.

**FIELD OF THE INVENTION**

This invention relates to photographic elements, processes and couplers, the couplers being of the type that release a photographically useful group (PUG) through a timing or linking group upon reaction with oxidized color developing agent during processing.

**BACKGROUND OF THE INVENTION**

Various ways are recognized in the photographic industry for releasing a PUG from a compound, such as a coupler, in a photographic material and process. Release can be direct, for example upon reaction of the coupler with oxidized color developing agent during processing, or it can be indirect through a linking or timing group. Linking and timing groups provide the ability to control the timing and rate of release of a PUG in a photographic element, as well as the rate and distance of diffusion of the PUG in the element during processing.

U.S. Pat. No. 4,248,962 describes compounds that release a PUG, such as a development inhibitor group, through a timing group which functions by an (intramolecular) nucleophilic displacement reaction. Other examples of compounds that are capable of releasing a PUG are described in U.S. Pat. Nos. 4,409,323 and 4,861,701. In U.S. Pat. No. 4,409,323, compounds are described which release a PUG by a mechanism which involves electron transfer down a conjugated chain. In U.S. Pat. No. 4,861,701, sequences of timing groups are utilized to release a PUG and to provide desirable control over the impact of the PUG on photographic properties.

European Patent Applications 0 499 279 and 0 438 129 describe photographic compounds having a heterocyclic timing nucleus attached to a coupler moiety through an —O—C(O)— or —OCH<sub>2</sub>— group, or other group capable of releasing the heterocyclic timing nucleus by electron transfer down an unconjugated chain followed by electron transfer down the conjugated chain of the heterocycle. However, these compounds do not provide a high degree of flexibility in their rate of release of a PUG, or in their synthetic design, as they are limited by the substituent groups on the heterocyclic timing or linking group.

A need exists for a photographic coupler that is synthetically simple to manufacture; that is capable of providing a wide range of release rates depending upon the particular selection of timing or linking groups and the substituents thereon; and that is stable when stored for prolonged periods, especially under tropical conditions. The coupler which is needed should be capable of releasing a PUG, such as a development inhibitor, providing effects including, for example, the reduction of gradation, the production of a finer color grain, the improvement of sharpness through the so-called edge effect and the improvement of color purity and color brilliance through so-called inter-image effects.

**SUMMARY OF THE INVENTION**

This invention provides a photographic element comprising a support having situated thereon at least one silver

## 2

halide emulsion layer, the element further comprising a photographic coupler represented by the formula



wherein

COUP is a coupler moiety having a coupling site to which T<sup>1</sup> is attached;

T<sup>1</sup> is a timing or linking group which releases from COUP during processing and which functions by electron transfer down a conjugated or unconjugated chain, or by a nucleophilic displacement reaction, to release T<sup>2</sup>;

T<sup>2</sup> is a triazole timing or linking group which, after release from T<sup>1</sup>, functions by a nucleophilic displacement reaction to release T<sup>3</sup> or PUG and is represented by the formula:



wherein \*\* denotes the point of attachment to T<sup>1</sup> and \*\*\* denotes the point of attachment to T<sup>3</sup> or PUG;

R<sup>1</sup> is a hydrogen or halogen atom, or an aliphatic, carbocyclic, carbamoyl, sulfamoyl, carbonamido, sulfonamido, alkoxy carbonyl, alkyl or arylketo, alkyl or arylsulfo, sulfo, hydroxy, acyl, nitro, cyano, amino, alkoxy, alkoxyalkyl, aryloxy, aryloxyalkyl, thioalkoxy, thioalkoxyalkyl, thioaryloxy, thioaryloxyalkyl or heterocyclic group;

X<sup>2</sup> is a linking group which spatially relates a nitrogen atom of the triazole ring and E<sup>2</sup> so that upon displacement of T<sup>2</sup> from T<sup>1</sup>, T<sup>2</sup> undergoes a nucleophilic displacement reaction with the formation of a three to eight-membered ring and the cleavage of the bond between E<sup>2</sup> and PUG or T<sup>3</sup>;

E<sup>2</sup> is an electrophilic group which is attached to T<sup>3</sup> or PUG and which is displaced therefrom by said nucleophilic displacement reaction after T<sup>2</sup> is displaced from T<sup>1</sup>;

T<sup>3</sup> is a timing or linking group attached to E<sup>2</sup> which is released therefrom after T<sup>2</sup> releases from T<sup>1</sup>, and which functions by electron transfer down a conjugated or unconjugated chain, or by a nucleophilic displacement reaction, to release PUG;

b and c are independently selected from 0 or 1; and

PUG is a photographically useful group.

In one useful embodiment b is 0. This invention further provides a coupler as described above.

The invention provides the opportunity to achieve improved image modification in photographic elements through the use of a new type of coupler in a silver halide photographic element, which coupler is capable of releasing a PUG upon photographic processing. The new coupler is synthetically simple to manufacture and provides improved release rates over previously known PUG releasing couplers

containing a heterocyclic timing or linking group. The coupler provides greater flexibility in the selection of timing or linking groups and the substituents thereon, and is stable under various types of storage conditions. The coupler utilized in the invention, particularly when PUG is a development inhibitor, provides improved interlayer interimage effects and acutance levels in photographic elements in which it is contained.

#### DETAILED DESCRIPTION OF THE INVENTION

In the photographic coupler utilized in the present invention, the coupler moiety, as represented by COUP, can be any moiety that will react with oxidized color developing agent during processing to cleave the bond between T<sup>1</sup> or T<sup>2</sup> and the coupler moiety. The coupler moiety as described herein includes conventional coupler moieties employed to yield both colorless and colored products upon reaction with oxidized color developing agents. Both types of coupler moieties are well known to those skilled in the photographic art and are exemplified in, for example, *Research Disclosure*, September 1994, Item 36544, all published by Kenneth Mason Publications, Ltd., Dudley Annex, 12a North Street, Emsworth, Hampshire PO10 7DQ, ENGLAND.

The coupler moiety can be ballasted or unballasted, and if unballasted, the dye formed upon oxidative coupling is capable of diffusing throughout, or being washed out of, the photographic element (sometimes known as a washout coupler). The coupler can be monomeric, or it can be part of a dimeric, oligomeric or polymeric coupler, in which case more than one PUG can be contained in the coupler. The coupler can also form part of a bis compound in which the PUG forms part of a link between two coupler moieties.

Representative coupler moieties suitable for use in the invention are as follows:

A. Couplers which form cyan dye upon reaction with oxidized color developing agent are described in such representative patents and publications as: U.S. Pat. Nos. 2,772,162; 2,895,826; 3,002,836; 3,034,892; 2,474,293; 2,423,730; 2,367,531; 3,041,236; 4,333,999 and "Farbkuppler-eine Literaturubersicht," published in Agfa Mitteilungen, Band III, pp. 156-175 (1961), all of which are incorporated herein by reference.

Preferably such cyan dye-forming couplers are phenols and naphthols.

B. Couplers which form magenta dye upon reaction with oxidized color developing agent are described in such representative patents and publications as: U.S. Pat. Nos. 2,600,788; 2,369,489; 2,343,703; 2,311,082; 3,152,896; 3,519,429; 3,062,653; 2,908,573 and "Farbkuppler-eine Literaturubersicht," published in Agfa Mitteilungen, Band III, pp. 126-156 (1961), all of which are incorporated herein by reference.

Preferably such magenta dye-forming couplers are pyrazolones or pyrazolotriazoles. Such couplers are utilized in one preferred embodiment of this invention.

C. Couplers which form yellow dye upon reaction with oxidized color developing agent are described in such representative patents and publications as: U.S. Pat. Nos. 2,875,057; 2,407,210; 3,265,506; 2,298,443; 3,048,194; 3,447,928 and "Farbkuppler-eine Literaturubersicht," published in Agfa Mitteilungen, Band III, pp. 112-126 (1961), all of which are incorporated herein by reference.

Preferably such yellow dye-forming couplers are acylacetamides, such as benzoylacetamides and pivaloylacetamides.

D. Couplers which form a colorless product upon reaction with an oxidized color developing agent are described in such representative patents as: U.K. Patent No. 861,138; and U.S. Pat. Nos. 3,632,345; 3,928,041; 3,958,993 and 3,961,959, all of which are incorporated herein by reference.

Specific representative examples of coupler moieties suitable for use in the invention are as follows:



## 5



Formula (1J)

Formula (1K)

p in the above formulae can be 0 to 4; q can be 0 to 3; and r can be 0 to 5. The free bond in each of the coupler moieties described above represents the coupling site, which is the position to which the coupling-off group is linked. In the above formulae,  $R^{1a}$ ,  $R^{1b}$ ,  $R^{1c}$ ,  $R^{1d}$ ,  $R^{1e}$ ,  $R^{1f}$ ,  $R^{1g}$ ,  $R^{1h}$ ,  $R^{1i}$ ,  $R^{1j}$ , or  $R^{1k}$  may contain one or more solubilizing groups which will enable the coupler, upon reaction with oxidized color developing agent, to washout of the photographic element. Additionally,  $R^{1h}$  and  $R^{1i}$  can be a hydrogen. Such groups, and couplers containing them, are exemplified in U.S. Pat. Nos. 4,482,629; 5,026,628; 5,151,343; 5,250,398; and 5,250,399, which are incorporated herein by reference. Specifically preferred solubilizing groups are selected from a carboxyl, sulfo, carbonamido or hydroxyl group, or salt thereof. It is preferred that when a solubilizing group is present, the coupler moiety is also unballasted so that complete washing out of the dye can occur. By unballasted, it is meant that each  $R^{1a}$  to  $R^{1k}$  contain no more than 20 carbon atoms, preferably no more than 12 carbon atoms, and optimally no more than 8 carbon atoms.

$R^{1a}$  to  $R^{1k}$ , p, q and r in formulae (1A) to (1K) are set forth in more detail as follows. Each of  $R^{1a}$  to  $R^{1k}$  is independently selected from the group consisting of a substituted or unsubstituted aliphatic, carbocyclic or heterocyclic group. Aliphatic, carbocyclic, and heterocyclic groups as used herein and elsewhere in this specification are defined in accordance with the definitions set forth in Grant and Hackh's *Chemical Dictionary*, fifth ed., McGraw-Hill 1987, and are in accordance with general rules of chemical nomenclature. The following descriptions of exemplary aliphatic, carbocyclic and heterocyclic groups are intended to be utilized throughout this application unless specifically noted otherwise.

Exemplary aliphatic groups include alkyl, alkene, and alkyne groups, particularly those having 1 to 25 carbon atoms. Examples of useful groups include methyl, ethyl, propyl, butyl, pentyl, hexyl, octyl, nonyl, decyl, dodecyl, hexadecyl, octadecyl, isopropyl, t-butyl, butenyl, pentenyl, hexenyl, octenyl, dodecenyl, propynyl, butynyl, pentynyl, hexynyl, and octynyl.

Exemplary carbocyclic groups (which include aryl groups) are those having a cyclic portion of 4 to 10 carbon atoms. Examples of useful groups include phenyl, tolyl, naphthyl, cyclohexyl, cyclopentyl, cyclohexenyl, cycloheptatrienyl, cyclooctatrienyl, cyclononatrienyl, cyclopentenyl, anilinyl, and anisidinyl.

Exemplary heterocyclic groups (which include heteroaryl groups) are those in which the cyclic portion has 5 to 10 atoms. Examples of useful groups include pyrrolyl, furyl, tetrahydrofuryl, pyridyl, picolinyl, piperidinyl, morpholinyl, thiadiazolyl, thiatriazolyl, benzothiazolyl, benzoxazolyl, benzimidazolyl, benzoselenozolyl, indazolyl, quinolyl, quinaldiny, pyrrolidinyl, thiophenyl, oxazolyl, thiazolyl, imidazolyl, selenazolyl, tellurazolyl, triazolyl, tetrazolyl, oxadiazolyl, thienyl, pryanyl, chromenyl, isothiazolyl, isoxazolyl, pyrazinyl, pyrimidinyl, pyridazinyl, indolyl, purinyl, isoquinolyl, quinoxaliny, and quinazoliny. Preferred heteroatoms are nitrogen, oxygen, and sulfur.

## 6

It is understood throughout this specification and claims that any reference to a substituent by the identification of a group or a ring containing a substitutable hydrogen (e.g., alkyl, amine, aryl, alkoxy, heterocyclic, etc.), unless otherwise specifically described as being unsubstituted or as being substituted with only certain substituents, shall encompass not only the substituent's unsubstituted form but also its form substituted with any substituents which do not negate the advantages of this invention. Also, reference to heterocyclic groups includes attachment at any position on the heterocycle. The term lower alkyl used herein means 1 to 5 carbon atoms. The term carbocyclic or heterocyclic group or ring, unless otherwise indicated, includes bicyclic or other fused rings. Groups suitable for substitution, which themselves may be substituted, include, but are not limited to, alkyl groups (for example, methyl, ethyl, hexyl), fluoralkyl groups (for example, trifluoromethyl), alkoxy groups (for example, methoxy, ethoxy, octyloxy), aryl groups (for example, phenyl, naphthyl, tolyl), hydroxy groups, halogen groups, aryloxy groups (for example, phenoxy), alkylthio groups (for example, methylthio, butylthio), arylthio groups (for example, phenylthio), acyl groups (for example, acetyl, propionyl, butyryl, valeryl), sulfonyl groups (for example, methylsulfonyl, phenylsulfonyl), ureido groups, carbamoyl groups, carbonamido groups, sulfamoyl groups, sulfonamido groups, acyloxy groups (for example, acetoxy, benzoxy), carboxy groups, cyano groups, sulfo groups, nitro groups and amino groups.

Preferred coupler moieties suitable for the couplers utilized in the invention are represented by



wherein \* denotes the coupling site to which  $T^1$  is attached.

$R^9$  is selected from hydrogen, or an aliphatic, carbocyclic, or heterocyclic group. In one embodiment this is a wash-out coupler and  $R^9$  is preferably hydrogen, an alkyl group containing 1 to 5 carbon atoms, an aryl group containing 6 to 10 carbon atoms or a heterocyclic group containing 4 to 8 carbon atoms. In another embodiment  $R^9$  is a ballast group which may contain the above groups.

$V_j$  is independently selected from an alkyl, heterocyclic, halo, carbamoyl, sulfamoyl, carbonamido, sulfonamido, keto, sulfo, nitro, hydroxyl, carboxyl, amino, alkoxy, alkoxy carbonyl, aryloxy, or arylthio, group; and preferably from an alkyl containing 1 to 5 carbon atoms or a carbamoyl, sulfamoyl, carbonamido, sulfonamido, sulfo, nitro, hydroxyl, carboxyl, amino, alkoxy or alkoxy carbonyl group.  $j$  is 0, 1, 2, 3, or 4, preferably 0 or 1.

Also preferred are coupler moieties represented by



wherein \* denotes the coupling site to which  $T^1$  is attached.

$R^{10}$  is selected from an aliphatic, carbocyclic, or heterocyclic group; and preferably from an alkyl group containing 1 to 10 carbon atoms, an aryl group containing 6 to 10 carbon atoms or a heterocyclic group containing 4 to 10 atoms;

Y is independently selected from an alkyl, heterocyclic, halo, carbamoyl, sulfamoyl, carbonamido, sulfonamido, keto, sulfo, nitro, hydroxyl, carboxyl, amino, alkoxy, alkoxy carbonyl, aryloxy or arylthio group. In one embodiment the coupler is preferably a wash-out coupler and Y is preferably an alkyl group containing 1 to 5 carbon atoms, carbamoyl, sulfamoyl, carbonamido, sulfonamido, sulfo, nitro, hydroxyl, carboxyl, amino, alkoxy or alkoxy carbonyl group. p is 0, 1, 2, 3, or 4, preferably 1 or 2. In another embodiment Y is a ballast group which may contain the above groups.

Other preferred coupler moieties are represented by



wherein \* denotes the coupling site to which T<sup>1</sup> is attached.

R<sup>13</sup> and R<sup>14</sup> are independently selected from a hydrogen atom, or an aliphatic, carbocyclic, heterocyclic, carbamoyl, sulfamoyl, carbonamido, sulfonamido, acyl, alkylsulfonyl, arylsulfonyl, alkylketo, arylketo, alkoxy carbonyl, aryloxy carbonyl, nitro, cyano, amino, alkoxy, alkoxyalkyl, aryloxy, aryloxyalkyl, thioalkoxy, thioalkoxyalkyl, thioaryloxy, or thioaryloxyalkyl group.

When R<sup>14</sup> is an amino group, preferred couplers are represented by



wherein R<sup>15</sup> an aliphatic, carbocyclic, or heterocyclic group.

The photographic coupler utilized in the invention reacts (i.e. couples) with the oxidized product of a color developing agent during processing to release (T<sup>1</sup>)<sub>b</sub>—T<sup>2</sup>—(T<sup>3</sup>)<sub>c</sub>—PUG.

T<sup>1</sup> and T<sup>3</sup> function as described below to release T<sup>2</sup> and PUG respectively. T<sup>2</sup> is a triazole linking or timing group. In this application reference is made to N-1 and N-2 of the triazole linking or timing group T<sup>2</sup>. N-1 is the nitrogen atom of the triazole ring to which T<sup>1</sup> or COUP is attached. N-2 is the nitrogen atom which, after release of T<sup>2</sup> from T<sup>1</sup>, is the nucleophile Nu<sup>2</sup>, which attacks E<sup>2</sup> to release T<sup>3</sup> or PUG.

The timing or linking group T<sup>2</sup> is shown by the formulae



wherein \*\* denotes the point of attachment to T<sup>1</sup> and \*\*\* denotes the point of attachment to T<sup>3</sup> or PUG;

Once released from T<sup>1</sup>, T<sup>2</sup> undergoes a nucleophilic reaction to release T<sup>3</sup> or PUG. This nucleophilic reaction is brought about when electron density shifts from the nitrogen atom N-1, of the triazole ring, onto the nitrogen atom N-2, which then acts as a nucleophile to attack the electrophile E<sup>2</sup>. This results in cleavage of the bond between T<sup>2</sup> and T<sup>3</sup>, when c is 1, or between T<sup>2</sup> and PUG, when c is 0. T<sup>2</sup> provides more flexibility to the coupler because both the ring and the X group may be substituted.

R<sup>1</sup> is selected from a hydrogen or halogen atom, or an aliphatic, carbocyclic, carbamoyl, sulfamoyl, carbonamido, sulfonamido, alkoxy carbonyl, alkyl or arylketo, alkyl or arylsulfo, sulfo, hydroxy, acyl, nitro, cyano, amino, alkoxy, alkoxyalkyl, aryloxy, aryloxyalkyl, thioalkoxy, thioalkoxyalkyl, thioaryloxy, thioaryloxyalkyl or heterocyclic group. Preferably R<sup>1</sup> is a hydrogen or halogen atom, an aliphatic group of 1 to 3 carbon atoms, or a carbamoyl or sulfamoyl group.

T<sup>1</sup> and T<sup>3</sup> can be any timing or linking groups known in the art, for instance those described below and in U.S. Pat.

20 Nos. 4,248,962; 4,409,323; 4,421,845; 4,857,447; 4,861,701; 4,864,604; 4,886,736; 4,891,304; 5,034,311; 5,055,385; 5,190,846; and European Patent Application 0 167 168, all of which are incorporated herein by reference. Thus, they independently may be timing or linking groups which function by nucleophilic displacement reaction (of the type described in, for example U.S. Pat. No. 4,248,962) or electron transfer down a conjugated chain (of the type described in, for example, U.S. Pat. No. 4,861,701). They may also be timing or linking groups which function by electron transfer down an unconjugated chain. These last 30 groups are known in the art under various names. Often they have been referred to as groups capable of utilizing a hemiacetal or iminoketal cleavage reaction or groups capable of utilizing a cleavage reaction due to ester hydrolysis. Regardless of their label, though, their mechanism is that 35 of electron transfer down an unconjugated chain which results, typically, in a relatively fast decomposition and the production of carbon dioxide, formaldehyde or other low molecular weight by-products. The groups are exemplified specifically in European Patent Application 0 464 612 and 0 40 523 451, both of which are incorporated herein by reference.

As used herein, "nucleophilic displacement reaction" means a reaction in which a nucleophilic center of a compound reacts directly, or indirectly, through an intervening molecule, with another site on the compound (an electrophilic center) to effect displacement of a group or atom attached to the electrophilic center. Such compounds have a nucleophilic group and electrophilic group spacially related by the configuration of the molecule to promote reactive proximity. The electrophilic group and the nucleophilic 45 group are located in the coupling-off group as described so that a cyclic organic ring, or a transient cyclic organic ring can be easily formed by an intramolecular reaction involving the nucleophilic center and the electrophilic center.

A nucleophilic group is understood to be a grouping of 50 atoms, one of which is electron rich. This atom is referred to as the nucleophilic center, representative examples of which include oxygen, sulfur and nitrogen atoms. An electrophilic group is understood to be a grouping of atoms, one or more of which is electron deficient. This atom(s) is referred to as 55 the electrophilic center, representative examples of which include carbonyl, thiocarbonyl, phosphinyl, and thiophosphinyl. Additional examples of nucleophilic groups, electrophilic groups and linking groups (to be discussed below) can be found in U.S. Pat. No. 4,248,962, incorporated herein 60 by reference.

In one preferred embodiment b is 0. In the image modifying couplers of this invention COUP may be directly

attached to the triazole timing or linking group. Such couplers generally exhibit more reactivity particularly when the triazole timing or linking group is attached to COUP through the N-1 nitrogen of the triazole group. In some suitable embodiments b is 0, c is 1; and T<sup>3</sup> is a timing or linking group which functions either by electron transfer down a conjugated chain or by a nucleophilic displacement reaction.

In another preferred embodiment of the invention, b and c are 1 and both T<sup>1</sup> and T<sup>3</sup> are timing or linking groups which function by nucleophilic displacement reactions. T<sup>1</sup> and T<sup>3</sup> may be the same or different.

In one embodiment of the invention, T<sup>1</sup> is a timing or linking group which functions by electron transfer down an unconjugated chain and T<sup>3</sup> is a timing or linking group which functions by electron transfer down a conjugated chain or T<sup>3</sup> is a timing or linking group which functions by nucleophilic displacement reaction.

In embodiments which involve nucleophilic displacement reactions of the timing or linking groups T<sup>1</sup>, T<sup>2</sup> or T<sup>3</sup>, subsequent discussions of the timing and linking groups will make reference to nucleophilic groups Nu<sup>1</sup> and Nu<sup>3</sup>, linking groups X<sup>1</sup>, X<sup>2</sup>, and X<sup>3</sup>, and electrophilic groups E<sup>1</sup>, E<sup>2</sup>, and E<sup>3</sup>. When describing T<sup>1</sup>, Nu<sup>1</sup>, X<sup>1</sup> and E<sup>1</sup> will be used; when describing T<sup>2</sup>, X<sup>2</sup> and E<sup>2</sup> will be used; and when describing T<sup>3</sup>, Nu<sup>3</sup>, X<sup>3</sup> and E<sup>3</sup> will be used. Nu<sup>1</sup> may be the same or different from Nu<sup>3</sup>; X<sup>1</sup>, X<sup>2</sup>, and X<sup>3</sup> may be the same or independently different from each other; and E<sup>1</sup>, E<sup>2</sup>, and E<sup>3</sup> may be the same or independently different from each other. Representative examples of nucleophilic groups, electrophilic groups and linking groups can be found in U.S. Pat. No. 4,248,962, previously incorporated by reference.

T<sup>1</sup> in these embodiments thus comprises a nucleophilic group (Nu<sup>1</sup>), which is attached to the coupling site of COUP and which is displaced therefrom upon reaction of COUP with oxidized color developing agent during processing. T<sup>1</sup> also comprises an electrophilic group (E<sup>1</sup>), which is attached to N-1 of the triazole moiety T<sup>2</sup>, and which is displaced therefrom by Nu<sup>1</sup> after Nu<sup>1</sup> is displaced from COUP.

T<sup>2</sup> comprises a triazole moiety with a masked nucleophilic group (N-2), which acts only as a nucleophile when T<sup>2</sup> is released from T<sup>1</sup> upon cleavage of the bond between E<sup>1</sup> and N-1. T<sup>2</sup> also comprised an electrophilic group (E<sup>2</sup>), which is attached to T<sup>3</sup> and which is displaced therefrom by N-2 after N-2 is unmasked as a nucleophile.

T<sup>3</sup> in these embodiments comprises a nucleophilic group (Nu<sup>3</sup>), which is attached to the electrophilic group E<sup>2</sup> of T<sup>2</sup> and which is displaced therefrom upon cleavage of the bond between E<sup>1</sup> and N-1, subsequent unmasking of N-2 as a nucleophile, and cleavage of the bond between E<sup>2</sup> and (Nu<sup>3</sup>). T<sup>3</sup> also comprises an electrophilic group (E<sup>3</sup>), which is attached to the PUG and which is displaced therefrom by Nu<sup>3</sup> after Nu<sup>3</sup> is displaced from T<sup>2</sup>.

The nucleophilic and electrophilic groups in T<sup>1</sup>, T<sup>2</sup> and T<sup>3</sup> are separated from each other by linking groups (X<sup>1</sup> in T<sup>1</sup>, X<sup>2</sup> in T<sup>2</sup> and X<sup>3</sup> in T<sup>3</sup>). The linking group X<sup>1</sup> spatially relates the nucleophilic group Nu<sup>1</sup> from the electrophilic group E<sup>1</sup> so that upon displacement of the nucleophilic group from the coupler moiety, T<sup>1</sup> undergoes a nucleophilic displacement reaction with the formation of, preferably, a three to eight membered ring and the cleavage of the bond between the electrophilic group E<sup>1</sup> and T<sup>2</sup>.

The linking group X<sup>2</sup> spatially relates the nucleophilic group N-2 of the triazole moiety, from the electrophilic group E<sup>2</sup> so that upon displacement of the triazole moiety and unmasking of the nucleophilic group from T<sup>1</sup>, T<sup>2</sup> undergoes a nucleophilic displacement reaction with the formation of, preferably, a three to eight membered ring

fused to the triazole moiety and cleavage of the bond between the electrophilic group E<sup>2</sup> and the nucleophilic group Nu<sup>3</sup>. Suitable X<sup>2</sup> linking groups include 1,2-phenylene, 1,2-naphthylene, pyridylene and —[(R<sup>3</sup>(R<sup>4</sup>)C)— as hereafter defined. Suitable E<sup>2</sup> electrophilic groups include —N(R<sup>7</sup>)C(O)— as hereafter defined.

The linking group X<sup>3</sup> spatially relates the nucleophilic group Nu<sup>3</sup>, from the electrophilic group E<sup>3</sup> so that upon displacement of the nucleophilic group from T<sup>2</sup>, T<sup>3</sup> undergoes a nucleophilic displacement reaction with the formation of, preferably, a three to eight membered ring and the cleavage of the bond between the electrophilic group E<sup>3</sup> and the PUG.

Preferred couplers utilized in the invention when T<sup>1</sup> functions by electron transfer down an unconjugated chain and T<sup>3</sup> functions by electron transfer down a conjugated chain are represented by the formula:



wherein COUP, T<sup>2</sup> and PUG are as defined previously.

In one suitable embodiment T<sup>1</sup> is a timing or linking group which functions by electron transfer down an unconjugated chain and is of the formula



wherein \* denotes the point of attachment of T<sup>1</sup> to COUP and \*\* denotes the point of attachment to T<sup>2</sup>. Z<sup>1</sup> is oxygen, sulfur or an unsubstituted or lower alkyl (C<sub>1</sub>-C<sub>5</sub>) substituted nitrogen. L<sup>1</sup> is a bivalent group selected from;



where R<sup>5</sup> and R<sup>6</sup> are independently a hydrogen, alkyl or an aryl group and are preferably hydrogen.

Preferably T<sup>1</sup> is selected from:



More preferably, T<sup>1</sup> is selected from:



$T^3$  is represented by the formula



5

wherein \*\*\* denotes the point of attachment to  $T^2$  and \*\*\*\* denotes the point of attachment to PUG.

W is oxygen, sulfur or an unsubstituted or lower alkyl ( $C_1-C_5$ ) substituted nitrogen. Q is independently selected from an alkyl, carbocyclic, heterocyclic, halo, carbamoyl, sulfamoyl, carbonamido, sulfonamido, keto, sulfo, nitro, hydroxyl, carboxyl, amino, alkoxy, alkoxy carbonyl, aryloxy, or arylthio group.  $Z^3$  represents the atoms necessary to complete a mono or bicyclic aromatic or heterocyclic ring system containing 5 to 10 ring atoms.  $—C(R^3)(R^4)—$  is in a favorable position relative to W, ortho or para, to allow for the conjugated transfer of electron density from W to  $—C(R^3)(R^4)—$  and cleavage of the bond between  $T^3$  and PUG. Preferably  $Z^3$  is a phenyl group.  $R^3$  and  $R^4$  are independently selected from hydrogen, or an aliphatic, carbocyclic, or heterocyclic group, or  $R^3$  and  $R^4$ , or  $R^3$  or  $R^4$  and  $Z^3$  together may form a 5, 6, or 7 membered carbocyclic or heterocyclic ring. By 5, 6 or 7 membered ring it is meant any of the carbocyclic or heterocyclic rings previously described that comprise the requisite number of carbon atoms in their ring structure.  $R^3$  and  $R^4$  are preferably independently selected from hydrogen or an alkyl having from 1 to 8 carbon atoms. n is 0, 1, 2 or 3.

Couplers utilized in another embodiment of the invention in which  $T^1$  functions by electron transfer down an unconjugated chain and  $T^3$  functions by a nucleophilic displacement reaction can be represented by the formula



wherein COUP,  $T^1$ ,  $T^2$ , and PUG are as defined previously.

$T^3$  is represented by the formula



wherein \*\*\* denotes the point of attachment to  $T^2$  and \*\*\*\* denotes the point of attachment to PUG.

$\text{Nu}^3$  is a nucleophilic group which is attached to  $T^2$  and which is displaced therefrom upon cleavage of the bond between  $T^1$  and  $T^2$ .  $X^3$  is a linking group for spatially relating  $\text{Nu}^3$  and  $E^3$  so that upon displacement of  $\text{Nu}^3$  from  $T^2$ ,  $\text{Nu}^3—X^3—E^3(T^3)$  undergoes a nucleophilic displacement reaction with the formation of a three to eight membered ring and the cleavage of the bond between  $E^3$  and the PUG.  $E^3$  is an electrophilic group which is attached to the PUG and which is displaced therefrom by  $\text{Nu}^3$  after  $\text{Nu}^3$  is displaced from  $T^2$ .

The preferred couplers utilized in this embodiment of the invention are represented by the formula



5

wherein COUP,  $T^1$ ,  $T^2$  and PUG are as previously defined and wherein  $\text{Nu}^3—X^3—E^3(T^3)$  is represented by the formula



10

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

788

792

796

800

804

808

812

816

820

824

828

832

836

840

844

850

854

860

864

868

872

876

880

884

888

892

896

900

904

908

912

916

920

924

930

934

940

944

948

952

956

960

964

968

972

976

980

984

988

992

996

1000

1004

1008

1012

1016

1020

1024

1028

1032

1036

1040

1044

1048

1052

1056

1060

1064

1068

1072

1076

1080

1084

1088

1092

1096

1100

1104

1108

1112

1116

1120

1124

1128

1132

1136

1140

1144

1148

1152

1156

1160

1164

1168

1172

1176

1180

1184

1188

1192

1196

1200

1204

1208

1212

1216

1220

1224

1228

1232

1236

1240

1244

1248

1252

1256

1260

1264

1268

1272

1276

1280

1284

1288

1292

1296

13



W, Q, n and R<sup>7</sup> are as defined above.

Couplers utilized in another embodiment of the invention in which both T<sup>1</sup> and T<sup>3</sup> function by nucleophilic displacement reactions can be represented by the formula



wherein COUP, T<sup>2</sup>, Nu<sup>3</sup>, X<sup>3</sup>, E<sup>3</sup> and PUG are as previously defined. T<sup>1</sup> is  $-\text{Nu}^1-\text{X}^1-\text{E}^1-$ . Nu<sup>1</sup> is a nucleophilic group which is attached to the coupling site of COUP and which is displaced therefrom upon reaction of COUP with oxidized color developing agent during processing. X<sup>1</sup> is a linking group for spatially relating Nu<sup>1</sup> and E<sup>1</sup> so that upon displacement of Nu<sup>1</sup> from COUP,  $-\text{Nu}^1-\text{X}^1-\text{E}^1-$  undergoes a nucleophilic displacement reaction with the formation of a three to eight membered ring and the cleavage of the bond between E<sup>1</sup> and T<sup>2</sup>. E<sup>1</sup> is an electrophilic group which is attached to T<sup>2</sup> and which is displaced therefrom by Nu<sup>1</sup> after Nu<sup>1</sup> is displaced from COUP. A more preferred embodiment is represented by



wherein COUP, T<sup>2</sup>, W, n, m, Q, Z<sup>3</sup>, R<sup>3</sup>, R<sup>4</sup>, R<sup>7</sup> and PUG are as previously defined.

In addition to the preferred timing and linking groups described above, some other suitable T<sup>1</sup> and T<sup>3</sup> groups can be selected from the following:

1. Acyclic timing or linking groups capable of nucleophilic displacement reaction:

14



where r<sup>1</sup> is 0 to 5; preferably 2, 3 or 4; Nu is a nucleophilic group, typically



and R<sup>8</sup> is hydrogen, or an aliphatic, carbocyclic, or heterocyclic group. Preferably, it is an alkyl of 1 to 20 carbon atoms or aryl of 6 to 20 carbon atoms. More preferably, it is an alkyl of 1 to 4 carbon atoms or an aryl of 6 to 10 carbon atoms.

2. Aromatic timing and linking groups capable of electron transfer down a conjugated chain:



30 where Z<sup>2</sup> is oxygen, sulfur or an unsubstituted or lower alkyl (C<sub>1</sub>-C<sub>5</sub>) substituted nitrogen; L<sup>2</sup> is pyridylene, 1,2- or 1,4-phenylene or naphthalene group; and R<sup>11</sup> and R<sup>12</sup> are independently selected from a hydrogen, or an alkyl or aryl group, preferably one containing fewer than 10 carbon atoms.

35 The coupler utilized in the invention releases a PUG precursor upon coupling during processing. The PUG can be any PUG known in the art. Examples include development inhibitors, bleach accelerators, development accelerators, 40 dyes, bleach inhibitors, couplers, developers, silver complexing agents, fixing agents, image toners, stabilizers, hardeners, tanning agents, fogging agents, ultraviolet radiation absorbers, antifoggants, nucleators, chemical or spectral sensitizers, and desensitizers. Other PUGs known in the art 45 are also possible in the present invention. These PUGs, as well as those specifically described above, can be released from  $-(\text{T}^1)_b-\text{T}^2-(\text{T}^3)_c-$  in the form of a precursor which, upon subsequent reaction, such as redox reaction 50 with a component of the developing solution, releases the PUG.

Couplers which release development inhibitors can enhance the effects heretofore obtained with untimed or unlinked DIR couplers since they can release a development inhibitor at a distance from the point at which oxidized color 55 developing agent reacted with the coupler, in which case they can provide, for example, enhanced interlayer interimage effects.

Couplers as described which release bleach inhibitors or 60 bleach accelerators can be employed in the ways described in the photographic art to inhibit the bleaching of silver or accelerated bleaching in areas of a photographic element.

Couplers as described which release a dye or dye precursor 65 can be used in processes where the dye is allowed to diffuse to an integral or separate receiving layer to form a desired image. Alternatively, the dye can be retained in the location where it is released to augment the density of the dye formed from the coupler from which it is released or to

modify or correct the hue of that dye or another dye. In another embodiment, the dye can be completely removed from the element and the dye which was not released from the coupler can be retained in the element as a color correcting mask.

Couplers as described in which the PUG is a developing agent can be used to release a developing agent which will compete with the color forming developing agent, and thus reduce dye density.

In the preferred embodiment of the invention the PUG is a development inhibitor. More preferably it is selected from a mercaptotetrazole, mercaptotriazole, dimercaptothiadiazole, mercaptooxadiazoles, mercaptoimidazole, mercaptobenzimidazole, mercaptobenzoxazole, mercaptobenzothiazole, mercaptothiadiazole, tetrazole, 1,2,3-triazole, 1,2,4-triazole or benzotriazole.

Representative PUGs suitable for use in the present invention can be found in the following references, all of which are incorporated herein by reference: U.S. Pat. Nos. 3,227,554; 3,384,657; 3,615,506; 3,617,291; 3,733,201 and U.K. Pat. No. 1,450,479 (development inhibitors); U.S. Pat. Nos. 3,880,658; 3,931,144; 3,932,380; 3,932,381;

16

3,942,987, and 4,840,884 (dye and dye precursors); *"On the Chemistry of White Couplers,"* by W. Puschel, Agfa-Gevaert AG Mitteilungen und der Forschungs-Laboratorium der Agfa-Gevaert AG, Springer Verlag, 1954, pp. 352-367; U.S.

- 5 Pat. Nos. 2,998,314; 2,808,329; 2,689,793; 2,742,832; German Pat. No. No. 1,168,769 and British Pat. No. 907,274 (couplers); U.S. Pat. Nos. 2,193,015; 2,108,243; 2,592,364; 3,656,950; 3,658,525; 2,751,297; 2,289,367; 2,772,282; 2,743,279; 2,753,256 and 2,304,953 (developing agents);  
10 U.S. Pat. Nos. 3,705,801; 3,715,208; and German OLS No. 2,405,279 (bleach inhibitors); U.S. Pat. Nos. 4,912,024; 5,063,145, columns 21-22, lines 1-70; and EP Pat. No. 0,193,389 (bleach accelerators); and U.S. Pat. Nos. 4,209, 580; 4,463,081; 4,471,045; and 4,481,287 and in published  
15 Japanese patent application No. 62-123,172 (electron transfer agents). Advantages of DIR couplers are described in, for example, the article by C. R. Barr, J. R. Thirtle and P. W. Vittum entitled "Development-Inhibitor-Releasing (DIR) Couplers in Color Photography" in Photographic Science and Engineering 13, 74(1969).

Specific couplers suitable for use in the invention are as follows:

### DIR Coupler, I-1:



I-1

### DIR Coupler, I-2:



I-2

-continued

### DIR Coupler, I-3:



I-3

### DIR Coupler, I-4:



I-4

### DIR Coupler, I-5:



I-5

### DIR Coupler, I-6:



J-6

-continued

DIR Coupler, I-7:



I-7

DIR Coupler, I-8:



I-8

DIR Coupler, I-9:



I-9

21

22

-continued

### DIR Coupler, I-10:



I-10

### DIR Coupler, I-11:



I-11

### Coupler, I-12:



I-12

-continued

Coupler, I-13:



I-13

### DIR Coupler, I-14:



I-14

DIR Coupler, I-15:



I-15

-continued

Coupler, I-16



Coupler, I-17:



DIR Coupler, I-18:



-continued



### DIR Coupler, I-20:



The photographic couplers can be incorporated in photographic elements by means and processes known in the photographic art. Photographic elements in which the couplers are incorporated can be simple elements comprising a support and a single silver halide emulsion layer or multilayer, multicolor elements. The couplers can be incorporated in at least one of the silver halide emulsion layers and/or in at least one other layer, such as an adjacent layer, where they will come into reactive association with oxidized color developing agent which has developed silver halide in the emulsion layer. Preferably the couplers are in a silver halide emulsion layer.

The silver halide emulsion layer can contain or have associated with it other photographic couplers such as dye-forming couplers, colored masking couplers, and/or competing couplers. These other photographic couplers can form dyes of any color and hue. Additionally, the silver halide emulsion layers and other layers of the photographic element can contain addenda conventionally contained in such layers.

A typical multilayer, multicolor photographic element can comprise a support having thereon a red-sensitive silver halide emulsion unit having associated therewith a cyan dye image-providing material, a green-sensitive silver halide emulsion unit having associated therewith a magenta dye image-providing material and a blue-sensitive silver halide emulsion unit having associated therewith a yellow dye image-providing material, at least one of the silver halide

40 emulsion units or another layer having associated therewith a photographic coupler as described above. Each silver halide emulsion unit can be composed of one or more layers and the various units and layers can be arranged in different locations with respect to one another.

45 The light sensitive silver halide emulsions can include coarse, regular or fine grain silver halide crystals or mixtures thereof, in a hydrophobic colloid, such as gelatin. The crystals can be comprised of any halide composition such as silver chloride, silver bromide, silver bromoiodide, silver 50 chlorobromide, silver chloroiodide, silver chlorobromoiodide and mixtures thereof. The emulsions can be negative-working or positive-working emulsions and can be incorporated into negative or reversal elements as described in U.S. Pat. No. 5,411,839, as well as other types of elements 55 known in the art. They can form latent images predominantly on the surface of the silver halide grains or predominantly on the interior of the silver halide grains. They can be chemically and spectrally sensitized by methods known in the art.

60 The photographic elements may also contain a transparent magnetic recording layer such as a layer containing magnetic particles on the underside of a transparent support, as described in U.S. Pat. Nos. 4,279,945 and 4,302,523 and in *Research Disclosure*, November 1992, Item 34390 published by Kenneth Mason Publications, Ltd., Dudley Annex, 12a North Street, Emsworth, Hampshire PO10 7DQ, ENGLAND. Typically, the element will have a total thick-

ness (excluding the support) of from about 5 to about 30 microns. Further, the photographic elements may have an annealed polyethylene naphthalate film base such as described in Hatsumei Kyoukai Koukai Gihou No. 94-6023, published Mar. 15, 1994 (Patent Office of Japan and Library of Congress of Japan) and may be utilized in a small format system, such as described in *Research Disclosure*, June 1994, Item 36230 published by Kenneth Mason Publications, Ltd., Dudley Annex, 12a North Street, Emsworth, Hampshire PO10 7DQ, ENGLAND, and such as the Advanced Photo System, particularly the Kodak ADVANTIX films or cameras.

The photographic elements can be incorporated into exposure structures intended for repeated use or exposure structures intended for limited use, variously referred to as single use cameras, lens with film, or photosensitive material package units.

The photographic elements can be exposed with various forms of energy which encompass the ultraviolet, visible, and infrared regions of the electromagnetic spectrum as well as with electron beam, beta radiation, gamma radiation, x-ray, alpha particle, neutron radiation, and other forms of corpuscular and wave-like radiant energy in either noncoherent (random phase) forms or coherent (in phase) forms, as produced by lasers. When the photographic elements are intended to be exposed by x-rays, they can include features found in conventional radiographic elements.

The photographic elements are preferably exposed to actinic radiation, typically in the visible region of the spectrum, to form a latent image, and then processed to form a visible dye image. Development is typically followed by the conventional steps of bleaching, fixing, or bleach-fixing, to remove silver or silver halide, washing, and drying.

In the following Table, reference will be made to (1) *Research Disclosure*, December 1978, Item 17643, (2) *Research Disclosure*, December 1989; Item 308119, and (3) *Research Disclosure*, September 1994, Item 36544, all published by Kenneth Mason Publications, Ltd., Dudley Annex, 12a North Street, Emsworth, Hampshire PO10 7DQ, ENGLAND, the disclosures of which are incorporated herein by reference. The Table and the references cited in the Table are to be read as describing particular components suitable for use in the elements of the invention. The Table and its cited references also describe suitable ways of preparing, exposing, processing and manipulating the elements, and the images contained therein. Photographic elements and methods of processing such elements suitable for use with this invention are described in *Research Disclosure*, February 1995, Item 37038, published by Kenneth Mason Publications, Ltd., Dudley Annex, 12a North Street, Emsworth, Hampshire PO10 7DQ, ENGLAND, the disclosure of which is incorporated herein by reference.

-continued

| Reference | Section         | Subject Matter                                        |
|-----------|-----------------|-------------------------------------------------------|
| 2         | VI              |                                                       |
| 3         | VII             |                                                       |
| 1         | VIII            | Absorbing and scattering                              |
| 2         | VIII, XIII, XVI | materials; Antistatic layers; matting agents          |
| 3         | VIII, IX C & D  |                                                       |
| 10        | VII             | Image-couplers and image-modifying couplers; Wash-out |
| 2         | VII             | couplers; Dye stabilizers and hue modifiers           |
| 3         | X               |                                                       |
| 1         | XVII            | Supports                                              |
| 2         | XVII            |                                                       |
| 3         | XV              |                                                       |
| 3         | XI              | Specific layer arrangements                           |
| 3         | XII, XIII       | Negative working emulsions; Direct positive emulsions |
| 20        | XVIII           | Exposure                                              |
| 3         | XVI             |                                                       |
| 1         | XIX, XX         | Chemical processing;                                  |
| 2         | XIX, XX, XXII   | Developing agents                                     |
| 3         | XVIII, XIX, XX  |                                                       |
| 3         | XIV             | Scanning and digital processing procedures            |

## SYNTHETIC EXAMPLES

The following synthetic examples illustrate the synthesis of couplers suitable for use in the invention. It is intended to be illustrative, and can be readily modified by one of ordinary skill in the art to obtain other suitable couplers.

## Synthesis of DIR Couplers I-1 and I-2.

## Intermediate A-3:

2-Chloro-N-[2-chloro-5-[(hexadecylsulfonyl)amino]phenyl]-4,4-dimethyl-3-oxo-pentanamide A-1, (6.5 g, 11.01 mMole), and 4-[2-(phenylamino)methyl-4-nitro]phenyl-5-phenyl-2H-1,2,3-triazole A-2, (4.5 g, 12.12 mMole), were suspended in acetonitrile (60 mL), treated with tetramethylguanidine (3.0 mL, 24.23 mL), and the resulting solution stirred at 25° C. for 30 minutes. At the end of this period the solution was diluted with ethyl acetate (150 mL) and washed with 2N-HCl (2×100 mL). The organic layer was then dried over MgSO<sub>4</sub>, filtered and concentrated under reduced pressure. The residue was dissolved in a mixture of ethyl acetate, methylene chloride and heptane in the ratio of 30:20:170 respectively and then chromatographed under medium pressure using a mixture of ethyl acetate and heptane in the ratio of 30:70 respectively. This gave the product A-3, yield 6.0 g.

## Intermediate A-4:

Intermediate A-3 (6.5 g, 7.01 mMole), was dissolved in dry tetrahydrofuran (50 mL), to which was added a 20% solution of phosgene in toluene (6.9 mL, 14.02 mMole), and the resulting solution was stirred at 25° C. for 15 minutes. The reaction solution was then concentrated under reduced pressure and the residue A-4, used as such in the next step of the sequence.

## 60 DIR Coupler I-1:

Intermediate A-4 (5.61 mMole), was dissolved in dry pyridine (50 mL) to which was added phenyl 1H-benzotriazole-5-carboxylate A-5, (1.34 g, 5.6 mMole), and the mixture was stirred at 25° C. for 3 hours. The reaction was then diluted with ethyl acetate (150 mL) and washed with 2N-HCl (2×100 mL). The organic layer was then dried over MgSO<sub>4</sub>, filtered and concentrated under

| Reference | Section                        | Subject Matter                                                                                    |
|-----------|--------------------------------|---------------------------------------------------------------------------------------------------|
| 1         | I, II                          | Grain composition,                                                                                |
| 2         | I, II, IX, X, XI, XII, XIV, XV | morphology and preparation. Emulsion preparation including hardeners, coating aids, addenda, etc. |
| 3         | I, II, III, IX A & B           |                                                                                                   |
| 1         | III, IV                        | Chemical sensitization and spectral sensitization/ desensitization                                |
| 2         | III, IV                        |                                                                                                   |
| 3         | IV V                           |                                                                                                   |
| 1         | V                              | UV dyes, optical brighteners, luminescent dyes                                                    |
| 2         | V                              |                                                                                                   |
| 3         | VI                             |                                                                                                   |
| 1         | VI                             | Antifoggants and stabilizers                                                                      |

31

reduced pressure. The residue was dissolved in a mixture of ethyl acetate, methylene chloride and heptane in the ratio of 20:10:80 respectively and then chromatographed under medium pressure, initially using the latter solvent mixture, and then changing to a mixture of ethyl acetate and heptane in the ratio of 40:160 respectively. This gave the product, DIR Coupler I-1, yield 6.0 g.

DIR Coupler I-2:

Intermediate A-4 (5.93 mMole), was dissolved in dry pyridine (60 mL) to which was added the sodium salt of phenyl mercaptotetrazole (1.30 g, 6.53 mMole) and the mixture was stirred at 25° C. for 30 minutes. The reaction was then diluted with ethyl acetate (150 mL) and washed with 2N-HCl (3x100 mL). The organic layer was then dried over MgSO<sub>4</sub>, filtered and concentrated under reduced pressure. The residue was dissolved in 25% ethyl acetate in heptane and chromatographed under medium pressure using the same solvent mixture. This gave the product, DIR Coupler I-2, yield 5.5 g.

The above synthesis is represented in following SCHEME 1:



32

-continued  
SCHEME 1



40 The following examples illustrate the practice of the invention. They are intended to be illustrative, and should not be construed as limiting the invention to the specific embodiments disclosed.

#### Examples

45 Photographic elements were prepared by coating the following layers on a cellulose acetate film support (amounts of each component are indicated in mg/m<sup>2</sup>):

|    |                     |                                                                                                                                                                                                                  |
|----|---------------------|------------------------------------------------------------------------------------------------------------------------------------------------------------------------------------------------------------------|
| 50 | Emulsion layer 1:   | Gelatin-2420; red sensitized silver bromoiodide (as Ag)-1615; magenta image coupler (Ma-1)-557 dispersed in tritolyl phosphate.<br>(RECEIVER LAYER)                                                              |
| 55 | Interlayer          | Gelatin-860; didodecylhydroquinone-113                                                                                                                                                                           |
| 55 | Emulsion layer 2:   | Gelatin-2690; green sensitized silver bromoiodide (as Ag)-1615; yellow image coupler (Ye-1)-694 dispersed in dibutyl phthalate; DIR coupler of Tables 1 and 2 dispersed in tritolyl phosphate.<br>(CAUSER LAYER) |
| 60 | Protective Overcoat | Gelatin-5380; bisvinylsulfonylmethyl ether at 2% total gelatin.                                                                                                                                                  |

33

Structures of couplers utilized in the Examples are as follows:

Magenta Image Coupler, Ma-1:



Yellow Image Coupler, Ye-1:



Control DIR Coupler, D-1:



Control DIR Coupler, D-2:



Strips of each element were exposed to a green or white light through a graduated density step tablet and then developed for 3.25 minutes at 38° C. in the following color

34

developer. Development was then stopped, and the elements washed, bleached, fixed, and dried.

| Ma-1 | Color Developer                                                 |         |
|------|-----------------------------------------------------------------|---------|
|      | 5                                                               | 800 mL  |
|      | Distilled water                                                 | 800 mL  |
|      | Sodium Sulfite, anhydrous                                       | 0.38 g  |
|      | CD-4' (color developer)*                                        | 4.52 g  |
|      | Potassium Carbonate, anhyd.                                     | 34.3 g  |
|      | Potassium Bicarbonate                                           | 2.32 g  |
|      | Sodium Bromide                                                  | 1.31 g  |
|      | Potassium Iodide                                                | 1.20 mg |
|      | Hydroxylamine Sulfate                                           | 2.41 g  |
|      | Diethylenetriaminepentacetic acid, pentasodium salt (40% Soln.) | 8.43 g  |
|      | Distilled water                                                 | to 1L   |
|      | Adjust pH to 10.0.                                              |         |

\*CD-4' is a KODAK color developer in which the active component is 4-amino-3-methyl-N-ethyl-N-beta-hydroxy-ethylaniline sulfate.

Photographic effects were determined as follows: A series of elements as described above containing no DI(A)R coupler or varying levels of DI(A)R coupler were exposed with green light. The contrast ( $\gamma$ ) along the straight line portion of each elements' D log H curve was measured. A plot of log ( $\gamma$ ) versus amount of DIR coupler ( $\mu$ moles) was made for each element (each element containing a different DI(A)R coupler). From these plots, the amount of DIR coupler needed to achieve log (0.7 $\gamma_o$ ) was read, where  $\gamma_o$  represented the contrast of the element containing no DI(A)R coupler. This value is recorded in the Table 1 as Level\* (\* amount of DIR coupler need to reduce the contrast by 30%).

Interlayer interimage effects representing the degree of color correction capable of being obtained by practice of the invention were evaluated after the same series of photographic elements were exposed to white light. The log of the causer contrast ( $\gamma_c$ ) and the log of the receiver contrast ( $\gamma_r$ ) were read for each of the DIR levels in the elements and a plot of log ( $\gamma_c$ ) versus log ( $\gamma_r$ ) was made. From this plot, ( $\gamma_r$ ) was determined at log (0.7 $\gamma_o$ ), where log (0.7 $\gamma_o$ ) was measured along the causer axis in the plot. The ratio ( $\gamma_c$ )/( $\gamma_r$ ) is recorded in Table 1 as Interlayer Interimage.

TABLE 1

| D-1 | DIR Coupler | Level* ( $\mu$ g/m <sup>2</sup> ) | Interlayer Interimage   |                               |
|-----|-------------|-----------------------------------|-------------------------|-------------------------------|
|     |             |                                   | Contrast ( $\gamma_c$ ) | ( $\gamma_c$ )/( $\gamma_r$ ) |
| 40  | D-1         | 215.2                             | 1.12                    | 0.72                          |
|     | I-1         | 150.6                             | "                       | 0.71                          |
|     | D-2         | 204.4                             | "                       | 0.45                          |
|     | I-2         | 107.6                             | "                       | 0.46                          |
|     | I-3         | 75.3                              | "                       | 0.48                          |

\*Amount of DIR coupler coated that is needed to reduce contrast 30%

As the data in Table 1 demonstrates, the couplers utilized in the present invention are more active than comparative compounds D-1 and D-2. They can thus be coated in photographic emulsions at lower levels than the comparative compounds, thus minimizing the potential that they will react with other components in the emulsion and adversely affect photographic performance.

TABLE 2

| DIR Coupler | % $\gamma$ Reduction<br>at 53.8 m<br>$\mu$ Moles/m <sup>2</sup> | % $\gamma$ Reduction<br>at 107.6 m<br>$\mu$ Moles/m <sup>2</sup> | % $\gamma$ Reduction<br>at 161.4 m<br>$\mu$ Moles/m <sup>2</sup> | 5  |
|-------------|-----------------------------------------------------------------|------------------------------------------------------------------|------------------------------------------------------------------|----|
| D-1         | 4                                                               | 14                                                               | 20                                                               |    |
| I-1         | 10                                                              | 22                                                               | 31                                                               |    |
| D-2         | 5                                                               | 15                                                               | 22                                                               |    |
| I-2         | 18                                                              | 32                                                               | 39                                                               |    |
| I-3         | 27                                                              | 53                                                               | 56                                                               | 10 |

Table 2, based on the Example provided above, shows the percentage change in contrast ( $\gamma$ ) for a given amount of each inventive or comparative coupler. As can be seen, the activity of the couplers utilized in the invention is far superior to that of the comparative couplers.

The invention has been described in detail with particular reference to preferred embodiments thereof, but it will be understood that variations and modifications can be effected within the spirit and scope of the invention.

What is claimed is:

1. A photographic coupler represented by the formula:



25

wherein

COUP is a coupler moiety having a coupling site to which  $\text{T}^1$  is attached;

$\text{T}^1$  is a timing or linking group which releases from COUP during processing and which functions by electron transfer down a conjugated or unconjugated chain, or by a nucleophilic displacement reaction, to release  $\text{T}^2$ ;

$\text{T}^2$  is a triazole timing or linking group which, after release from  $\text{T}^1$ , functions by a nucleophilic displacement reaction to release  $\text{T}^3$  or PUG and is represented by the formula:



30

35

40

wherein \*\* denotes the point of attachment to  $\text{T}^1$  and \*\*\* denotes the point of attachment to  $\text{T}^3$  or PUG;

$\text{R}^1$  is a hydrogen or halogen atom, or an aliphatic, carbocyclic, carbamoyl, sulfamoyl, carbonamido, sulfonamido, alkoxy carbonyl, alkyl or arylketo, alkyl or arylsulfo, sulfo, hydroxy, acyl, nitro, cyano, amino, alkoxy, alkoxyalkyl, aryloxy, aryloxyalkyl, thioalkoxy, thioalkoxyalkyl, thioaryloxy, thioaryloxyalkyl or heterocyclic group;

$\text{X}^2$  is a linking group which spatially relates a nitrogen atom of the triazole ring and  $\text{E}^2$  so that upon displacement of  $\text{T}^2$  from  $\text{T}^1$ ,  $\text{T}^2$  undergoes a nucleophilic displacement reaction with the formation of a three to eight membered ring and the cleavage of the bond between  $\text{E}^2$  and PUG or  $\text{T}^3$ ;

$\text{E}^2$  is an electrophilic group which is attached to  $\text{T}^3$  and which is displaced therefrom by said nucleophilic displacement reaction after  $\text{T}^2$  is displaced from  $\text{T}^1$ ;

$\text{T}^3$  is a timing or linking group attached to  $\text{E}^2$  which is released therefrom after  $\text{T}^2$  releases from  $\text{T}^1$ , and which functions by electron transfer down a conjugated or unconjugated chain, or by a nucleophilic displacement reaction, to release PUG;

$\text{b}$  and  $\text{c}$  are independently selected from 0 or 1; and

PUG is a photographically useful group.

2. The photographic coupler of claim 1 wherein  $\text{b}$  is 0.

